



US011532407B2

(12) **United States Patent**  
**Chen et al.**

(10) **Patent No.:** **US 11,532,407 B2**  
(b4) **Date of Patent:** **Dec. 20, 2022**

(54) **ALUMINUM CONDUCTOR ALLOYS HAVING IMPROVED CREEPING RESISTANCE**

(71) Applicant: **UNIVERSITE DU QUEBEC A CHICOUTIMI**, Saguenay (CA)

(72) Inventors: **Xiao-Grant Chen**, Saguenay (CA); **Lei Pan**, Saguenay (CA); **Kun Liu**, Saguenay (CA); **Alexandre Maltais**, Chicoutimi (CA); **Bruno Bourassa**, Jonqui  re (CA)

(73) Assignee: **UNIVERSITE DU QUEBEC A CHICOUTIMI**, Chicoutimi (CA)

(\*) Notice: Subject to any disclaimer, the term of this patent is extended or adjusted under 35 U.S.C. 154(b) by 808 days.

(21) Appl. No.: **16/319,100**

(22) PCT Filed: **Jul. 19, 2017**

(86) PCT No.: **PCT/CA2017/050868**

§ 371 (c)(1),  
(2) Date: **Jan. 18, 2019**

(87) PCT Pub. No.: **WO2018/014128**

PCT Pub. Date: **Jan. 25, 2018**

(65) **Prior Publication Data**

US 2021/0335516 A1 Oct. 28, 2021

**Related U.S. Application Data**

(60) Provisional application No. 62/365,020, filed on Jul. 21, 2016.

(51) **Int. Cl.**

**C22C 21/00** (2006.01)  
**H01B 1/02** (2006.01)

(52) **U.S. Cl.**  
CPC ..... **H01B 1/023** (2013.01); **C22C 21/00** (2013.01)

(58) **Field of Classification Search**  
CPC .. H01R 43/0207; H01R 43/048; H01R 4/183; H01R 4/188; H01R 4/62; H02G 15/076;  
(Continued)

(56) **References Cited**

**U.S. PATENT DOCUMENTS**

1,815,479 A \* 7/1931 Morell ..... C22C 18/02  
420/521  
3,668,019 A 6/1972 Hunsicker  
(Continued)

**FOREIGN PATENT DOCUMENTS**

CN 102912193 A 2/2013  
CN 103276257 A 9/2013  
(Continued)

**OTHER PUBLICATIONS**

Dec. 17, 2019—(MA) Preliminary Search Report—App 44561.  
(Continued)

*Primary Examiner* — Krystal Robinson

(74) *Attorney, Agent, or Firm* — Banner & Witcoff, Ltd.

(57) **ABSTRACT**

The present disclosure concerns aluminum conductor alloys having increased creep resistance, aluminum products comprising same and process using same. In some embodiments, the aluminum conductor alloy comprises, in weight percent: up to about 0.10 Si; up to about 0.5 Fe; up to about 0.30 Cu; between about 0.02 and about 0.1 Mg; up to about 0.04 B; and the balance being aluminum and unavoidable impurities.

**18 Claims, 11 Drawing Sheets**



(58) **Field of Classification Search**

CPC ..... H02G 15/14; H02G 9/12; C08K 5/5313;  
 H01B 1/02; H01B 1/023; C22C 21/00  
 USPC ..... 174/126.1  
 See application file for complete search history.

## FOREIGN PATENT DOCUMENTS

|    |             |          |
|----|-------------|----------|
| CN | 103667810 A | 3/2014   |
| CN | 104294090 A | 1/2015   |
| CN | 104294093 A | 1/2015   |
| CN | 105316535 A | 2/2016   |
| CN | 106893899 A | * 6/2017 |

## (56)

**References Cited**

## U.S. PATENT DOCUMENTS

|                   |         |                 |                         |
|-------------------|---------|-----------------|-------------------------|
| 4,182,640 A *     | 1/1980  | Yokota .....    | C22C 21/12<br>148/438   |
| 9,263,168 B2 *    | 2/2016  | Sekiya .....    | C22C 21/14              |
| 9,870,841 B2 *    | 1/2018  | Yoshida .....   | C22F 1/04               |
| 9,899,119 B2 *    | 2/2018  | Yoshida .....   | H01R 4/62               |
| 9,947,917 B2 *    | 4/2018  | Seki .....      | H01B 5/02               |
| 2002/0066503 A1 * | 6/2002  | Matsui .....    | C22C 9/00<br>148/432    |
| 2002/0162683 A1 * | 11/2002 | Fujiwara .....  | H01R 4/62<br>174/74 R   |
| 2008/0196923 A1 * | 8/2008  | Su .....        | C22C 21/00<br>174/110 R |
| 2012/0234427 A1 * | 9/2012  | Verboom .....   | C22C 21/04<br>138/143   |
| 2012/0234597 A1 * | 9/2012  | Madden .....    | H02G 15/076<br>174/74 R |
| 2013/0126055 A1   | 5/2013  | Sekiya et al.   |                         |
| 2013/0319585 A1 * | 12/2013 | Parson .....    | C22C 21/02<br>148/690   |
| 2014/0020796 A1   | 1/2014  | Sekiya et al.   |                         |
| 2014/0311769 A1 * | 10/2014 | In .....        | C22F 1/08<br>428/615    |
| 2015/0213913 A1 * | 7/2015  | Yoshida .....   | C22C 21/04<br>174/74 R  |
| 2015/0235729 A1 * | 8/2015  | Yoshida .....   | C22C 21/00<br>174/74 R  |
| 2018/0171439 A1 * | 6/2018  | Kobayashi ..... | H01B 7/00               |

## OTHER PUBLICATIONS

- Jan. 10, 2020—(CN) Office Action—App 201780045099.9.  
 Feb. 3, 2020—(EP) Supplemental Search Report—App 17830151.1.  
 Jan. 17, 2006, B. Raeisinia, W.J. Poole, D.J. Lloyd, Mater. “Examination of precipitation in the aluminum alloy AA6111 using electrical resistivity measurements” Sci. Eng. A 420, p. 245-249.  
 Feb. 9, 2013, C.J. Shi, W.M. Mao, X.G. Chen, “Evolution of activation energy during hot deformation of AA7150 aluminum alloy” Mater. Sci. Eng. A 571, p. 83-91.  
 May 22, 2003, E.A. Marquis, D.N. Seidman, D.C. Dunand, “Effect of Mg addition on the creep and yield behavior of an Al—Sc alloy” Acta Mater. 5, p. 4751-4760.  
 Dec. 19, 2000, F.J. Humphreys, J. “Review Grain and subgrain characterisation by electron backscatter diffraction” Mater. Sci. 36, p. 3833-3854.  
 Sep. 2016, L. Pan, K. Liu, F. Breton, X.-G. Chen, Abstract, “Effects of alloying elements on microstructure and creep properties of 8xxx aluminum conductor alloys”.  
 2011, “Standard Specification for 8000 Series Aluminum Alloy Wire for Electrical Purposes-Annealed and Intermediate Tempers” ASTM International B800-05.  
 Jul. 19, 2013, X.W. Wei, X.T. Zu, W.L. Zhou, “Compressive creep behaviour of Mg—Li—Al alloy” Mater. Sci. Tech. 22, p. 730-733.  
 Oct. 12, 2017—International Search Report and Written Opinion of PCT/CA2017/050868.

\* cited by examiner



**Figure 1a**



**Figure 1b**



**Figure 1c**



**Figure 1d**



Figure 2b



Figure 2a



Figure 3b



Figure 3a



Figure 4



Mg (wt.%) Figure 5b



Fe (wt.%) Figure 5c



Figure 7



Figure 6



Figure 8b



Figure 8a



Figure 9b



Figure 9a



Figure 10b



Figure 10a



Figure 10d



Figure 10c



Figure 11

## 1

**ALUMINUM CONDUCTOR ALLOYS  
HAVING IMPROVED CREEPING  
RESISTANCE**

**CROSS-REFERENCE TO RELATED  
APPLICATIONS AND DOCUMENTS**

This application is a U.S. National Phase filing of International Application No. PCT/CA2017/050868, filed on Jul. 19, 2017, which claims priority to U.S. provisional patent application No. 62/365,020 filed on Jul. 21, 2016, which prior applications are incorporated herewith by reference in their entireties.

**TECHNOLOGICAL FIELD**

The present disclosure concerns aluminum alloys that can be used as an electrical conductor material.

**BACKGROUND**

As the economy has developed in the past few decades, the demand for the electrical conductor materials has been significantly increasing. The 8xxx aluminum conductor alloys offer significant advantages such as low density, high conductivity to weight ratio and low cost over copper conductors. They progressively replace the copper conductor alloy in overhead transmission and distribution. For a wide application of aluminum conductors, it is necessary for them to satisfy the overall requirement of properties in electrical industry, notably the electrical conductivity, tensile strength and creep resistance. Consequently, considerable efforts have been devoted to develop the aluminum conductor alloys with high comprehensive properties.

Alloying of commercially pure aluminum alloy may create solid solution or individual phases that greatly improve tensile strength due to solid solution strengthening and precipitation strengthening. However, the electrical conductivity may drop because of the enhanced scattering of free electrons at solute atoms and precipitates. For electrical applications, it is a challenge to find a favourable combination of high electrical conductivity with enhanced mechanical properties in the alloy design and development.

In addition, creep property is one of the most important properties required in aluminum conductor alloys. Due to the Joule effect, temperature increase in the aluminum conductor and creep resistance is needed to avoid long term deformations.

It would be desirable to obtain an aluminum conductor alloy having improved creep resistance at relatively low temperatures without substantially decreasing its electrical conductivity. Alternatively or in combination, it would also be desirable to obtain an aluminum conductor alloy having improved cast properties.

**BRIEF SUMMARY**

The present disclosure concerns aluminum conductor alloys which, once cast, have improved creep resistance when compare to corresponding aluminum conductor alloys having less than 0.1 Mg (in weight percent).

In a first aspect, the present disclosure concerns aluminum conductor alloy having increased creep resistance. The aluminum conductor alloy comprises, in weight percent:

up to about 0.10 Si;  
up to about 0.5 Fe;  
up to about 0.30 Cu;

## 2

between about 0.02 and about 0.1 Mg;  
up to about 0.04 B;  
and the balance being aluminum and unavoidable impurities.

5 In an embodiment, the aluminum conductor alloy comprises up to about 0.05 Si. In another embodiment, the aluminum conductor alloy comprises between about 0.3 and about 0.5 Fe. In still another embodiment, the aluminum conductor alloy comprises between about 0.15 and about 0.30 Cu, for example, up to about 0.18 Cu. In still yet another embodiment, the aluminum conductor alloy comprises up to about 0.052 Mg or up to about 0.025 Mg. In yet another embodiment, the aluminum alloy comprises between about 0.001 and about 0.04 B. In a further, embodiment, the aluminum alloy has a secondary creep rate of  $1 \times 10^{-8} \text{ s}^{-1}$  or less when measured at  $100^\circ \text{C}$ . under a 69 MPa load.

10 In a second aspect, the present disclosure concerns a rod comprising the aluminum conductor alloy described herein.

15 In a third aspect, the present disclosure concerns an aluminum cast product comprising the aluminum conductor alloy described herein. The aluminum cast product can be, for example, a wire.

20 In a fourth aspect, the present disclosure concerns a process for improving the creep resistance of an aluminum product comprising a modified aluminum conductor alloy when compared to a corresponding aluminum product comprising a first aluminum conductor alloy. Broadly, the process comprises combining Mg with the first aluminum conductor alloy to provide the modified aluminum conductor alloy. The first aluminum conductor alloy comprises, in weight percent:

25 up to about 0.10 Si;  
up to about 0.5 Fe;  
up to about 0.30 Cu;  
up to about 0.04 B;  
and the balance being aluminum and unavoidable impurities.

30 In the process, the modified aluminum alloy comprises between about 0.02 and about 0.1 Mg. In an embodiment, the modified aluminum conductor alloy comprises up to about 0.05 Si. In another embodiment, the modified conductor aluminum alloy comprises between about 0.3 and about 0.5 Fe. In still another embodiment, the modified conductor aluminum alloy comprises between about 0.15 and about 0.30 Cu, such as, for example, up to about 0.18 Cu. In still another embodiment, the modified conductor aluminum alloy comprises up to about 0.052 Mg. In still

35 another embodiment, the modified conductor aluminum alloy comprises up to about 0.025 Mg. In yet another embodiment, the modified conductor aluminum alloy comprises between about 0.001 and about 0.04 B. In still yet another embodiment, the modified conductor aluminum alloy has a secondary creep rate of  $1 \times 10^{-8} \text{ s}^{-1}$  or less when measured at  $100^\circ \text{C}$ . under a 69 MPa load.

40 In a fifth aspect, the present disclosure provides an aluminum conductor alloy (also referred to as a modified aluminum alloy) obtainable or obtained by the process described herein. In an embodiment, the aluminum conductor alloy can be in the form of a rod.

45 In a sixth aspect, the present disclosure provides a process for making an aluminum product having improved creep resistance, the process comprising working the aluminum conductor alloy described herein, obtainable or obtained by the process described herein or the rod described herein in the aluminum product.

In a seventh aspect, the present disclosure provides an aluminum product obtainable or obtained by the process described herein. In an embodiment, the aluminum product can be a wire.

In the context of the present disclosure, the term "about" means that the recited numerical value is part of a range that varies within standard experimental error.

#### BRIEF DESCRIPTION OF THE DRAWINGS

Having thus generally described the nature of the invention, reference will now be made to the accompanying drawings, showing by way of illustration, a preferred embodiment thereof, and in which:

FIGS. 1A to D provide the optical micrographs showing the particles distribution of the alloys: (A) Al-0.3Fe, (B) Al-0.3Fe-0.29Cu, (C) Al-0.7Fe, and (D) Al-0.7Fe-0.18Cu-0.1Mg, showing fine Fe-rich intermetallic particles distributed along the extrusion direction (ED).

FIGS. 2A and B illustrate the evolution of subgrain size (in  $\mu\text{m}$ ) with increasing of (A) Cu ( $\blacksquare=\text{Al-0.3Fe-Cu}$ ;  $\square=\text{Al-0.5Fe-Cu}$ ;  $\blacktriangle=\text{Al-0.7Fe-Cu}$ ) and (B) Mg ( $\blacksquare=\text{Al-0.3Fe-0.18Cu-Mg}$ ;  $\square=\text{Al-0.5Fe-0.18Cu-Mg}$ ;  $\blacktriangle=\text{Al-0.7Fe-0.18Cu-Mg}$ ) contents of different alloys.

FIGS. 3A and B provide the individual influences of selected alloying elements on electrical conductivity (EC in % International Annealed Copper Standard, IACS): (A) Cu ( $\blacksquare=\text{Al-0.3Fe-Cu}$ ;  $\bullet=\text{Al-0.5Fe-Cu}$ ;  $\blacktriangle=\text{Al-0.7Fe-Cu}$ ) and (B) Mg ( $\blacksquare=\text{Al-0.3Fe-0.18Cu-Mg}$ ;  $\bullet=\text{Al-0.5Fe-0.18Cu-Mg}$ ;  $\blacktriangle=\text{Al-0.7Fe-0.18Cu-Mg}$ ).

FIG. 4 provides a correlation between calculated and experimental measured EC (in % IACS) for alloys Al-0.3Fe-Cu-Mg ( $\blacksquare$ ), Al-0.5Fe-Cu-Mg ( $\bullet$ ) and Al-0.7Fe-Cu-Mg ( $\blacktriangle$ ).

FIGS. 5A to C provide the individual influences of selected chemical elements on Ultimate Tensile Strength (UTS in MPa): (A) Cu ( $\blacktriangle=\text{Al-0.3Fe-Cu}$ ;  $\bullet=\text{Al-0.5Fe-Cu}$ ;  $\blacksquare=\text{Al-0.7Fe-Cu}$ ), (B) Mg ( $\blacksquare=\text{Al-0.3Fe-0.18Cu-Mg}$ ;  $\bullet=\text{Al-0.5Fe-0.18Cu-Mg}$ ;  $\blacktriangle=\text{Al-0.7Fe-0.18Cu-Mg}$ ), and (C) Fe with a linear relationship ( $\blacksquare=\text{Al-Fe}$ ;  $\bullet=\text{Al-0.29Cu-Fe}$ ;  $\blacktriangle=\text{Al-0.18Cu-0.1Mg-Fe}$ ).

FIG. 6 provides the correlation between calculated and experimental measured UTS (in MPa) for alloys ( $\blacksquare=\text{Al-0.3Fe-Cu-Mg}$ ;  $\bullet=\text{Al-0.5Fe-Cu-Mg}$ ;  $\blacktriangle=\text{Al-0.7Fe-Cu-Mg}$ ).

FIG. 7 provides the EC (in % IACS) and UTS (in MPa) profile of the alloys ( $\blacksquare/\blacksquare=\text{Al-0.3Fe-Cu-Mg}$ ;  $\blacksquare/\oplus=\text{Al-0.5Fe-Cu-Mg}$ ;  $\blacktriangle/\blacktriangle=\text{Al-0.7Fe-Cu-Mg}$ ) with different Cu and Mg additions. Arrows show the increasing Cu and Mg additions to their corresponding regions.

FIGS. 8A and B provide the typical compressive creep strain ( $\epsilon$ ) (A) and instantaneous creep rate ( $\dot{\epsilon}$ ) (B) curves of Al-0.3Fe alloys with Cu addition ( $\blacksquare=\text{Al-0.3Fe (base)}$ ;  $\square=\text{Al-0.3Fe-0.18Cu}$ ;  $\blacktriangle=\text{Al-0.3Fe-0.29Cu}$ ), tested at 100° C. and applied load of 69 MPa.

FIGS. 9A and B provide the typical compressive creep strain ( $\epsilon$  in %) (A) and instantaneous creep rate ( $\dot{\epsilon}$  in  $\text{s}^{-1}$ ) (B) curves (B) of Al-0.3Fe-0.18Cu alloys with Mg addition ( $\blacksquare=\text{Al-0.3Fe-0.18Cu}$ ;  $\bullet=\text{Al-0.3Fe-0.18Cu-0.025Mg}$ ;  $\blacktriangle=\text{Al-0.3Fe-0.18Cu-0.052Mg}$ ;  $\blacktriangledown=\text{Al-0.3Fe-0.18Cu-0.1Mg}$ ), tested at 100° C. and applied load of 69 MPa.

FIGS. 10A to D provide plots illustrating the variation of (A)-(B) the primary creep strain ( $\epsilon_p$  in %) and (C)-(D) minimum creep rate ( $\dot{\epsilon}_m$  in  $\text{s}^{-1}$ ) with increasing Cu content ((A) and (C)  $\blacksquare=\text{Al-0.3Fe-Cu}$ ;  $\bullet=\text{Al-0.5Fe-Cu}$ ;  $\blacktriangle=\text{Al-0.7Fe-Cu}$ ;  $\blacksquare/\blacksquare=\text{Al-0.3Fe-Cu-Mg}$ ;  $\blacksquare/\oplus=\text{Al-0.5Fe-Cu-Mg}$ ;  $\blacktriangle/\blacktriangle=\text{Al-0.7Fe-Cu-Mg}$ ), tested at 100° C. and applied load of 69 MPa.

FIGS. 11A to D provide plots illustrating the variation of (A)-(B) the primary creep strain ( $\epsilon_p$  in %) and (C)-(D) minimum creep rate ( $\dot{\epsilon}_m$  in  $\text{s}^{-1}$ ) with increasing Cu content ((A) and (C)  $\blacksquare=\text{Al-0.3Fe-Cu}$ ;  $\bullet=\text{Al-0.5Fe-Cu}$ ;  $\blacktriangle=\text{Al-0.7Fe-Cu}$ ;  $\blacksquare/\blacksquare=\text{Al-0.3Fe-Cu-Mg}$ ;  $\blacksquare/\oplus=\text{Al-0.5Fe-Cu-Mg}$ ;  $\blacktriangle/\blacktriangle=\text{Al-0.7Fe-Cu-Mg}$ ), tested at 100° C. and applied load of 69 MPa.

0.7Fe-Cu) and increasing Mg content ((B) and (D)  $\blacksquare=\text{Al-0.3Fe-0.18Cu-Mg}$ ;  $\bullet=\text{Al-0.5Fe-0.18Cu-Mg}$ ;  $\blacktriangle=\text{Al-0.7Fe-0.18Cu-Mg}$ ).

5 FIG. 11 provides the bar (ingot) temperature (in ° C.) in function of the Fe content of the alloys.

#### DETAILED DESCRIPTION

The present disclosure concerns the use of Mg in aluminum conductor alloys to increase creep resistance without substantially decreasing the electrical conductivity of the product comprising the aluminum conductor alloy. In some embodiments, the increase in creep resistance is observed at low temperatures (e.g.,  $\leq 0.4$  temperature melting point or 15  $T_m$ ). In some embodiments, the aluminum conductor alloys can also have a reduced Fe content which will facilitate casting operations without substantially decreasing the strength properties of the product comprising the aluminum conductor alloy.

20 In the context of the present disclosure, Mg can be added, at a weight percentage of between about 0.02 and 0.1 (in weight percent) to any aluminum conductor alloys to increase the creep resistance of said aluminum conductor alloy and without substantially decreasing the electrical 25 conductivity of said aluminum conductor alloy. In an embodiment, the addition of Mg can be coupled with a decrease in the Fe content the aluminum conductor alloy of the present disclosure can be limited to 0.5 or even 0.3 (in weight percent). For example, Mg can be added to the 30 wrought alloys of the 8xxx series (such as, for example, the aluminum alloys of the 8030 series) and to the wrought alloy of the 1xxx series (such as, for example, the aluminum alloys of the 1350 series).

35 One of the advantages of the aluminum conductor alloys 35 of the present disclosure is that, once cast, they exhibit increased creeping resistance when compared to another aluminum conductor alloy comprising less than 0.02 Mg (in weight percent). Since the aluminum conductor alloys of the present disclosure are intended to be used at low temperatures, this increase in creep resistance is preferably observed 40 at low temperatures (e.g.,  $\leq 0.4 T_m$  of the aluminum conductor alloy). In an embodiment, the increase in creep resistance occurs at temperatures between about 20° C. to about 200° C. or between about 50° C. to about 150° C. As it is known in the art, creep is characterized by three stages: primary, secondary and tertiary creep. During the primary creep, strain rates are relatively high, but reduce over time. During secondary creep, strain rates are stable. Secondary creep strain rates are typically used to characterize the 45 "creep strain rate" of a material, such as an aluminum conductor alloy. During tertiary creep, necking occurs which leads to failure of the alloy. Creep can be determined by the absolute strain measured or the strain rate measured. In an embodiment, an aluminum product made from the aluminum conductor alloy of the present disclosure (when compared to a corresponding aluminum product made from an aluminum conductor alloy having no deliberate addition of Mg or having less than 0.02 Mg (in weight percent)) has a 50 decreased minimum creep rate (e.g. the average creep rate during the secondary creep) or secondary creep rate, a decreased short-term creep deformation or primary creep rate, a decreased typical compressive creep strain and/or a decreased instantaneous creep rate. In some embodiments, the aluminum conductor alloys of the present disclosure have a secondary creep rate of at most (e.g., a maximal secondary creep rate) about  $1 \times 10^{-8}/\text{s}$  when measured at 55 100° C. under a 69 MPa load. The aluminum conductor 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090

alloys described herein have at most 0.1 Mg (in weight percent) in other to preserve the electrical conductivity of the alloy.

A further advantage of some of the aluminum conductor alloys of the present disclosure is that, if they comprise 0.5 Fe (in weight percent) or less (such as, for example less than about 0.5 or less than about 0.3 Fe, in weight percent), the aluminum conductor alloy will have improved casting properties, e.g., it will be easier and/or faster to cast (when compared to corresponding aluminum conductor alloys having more than 0.5 Fe, in weight percent).

Because the aluminum conductor alloys of the present disclosure are intended to be used as electrical conductor material, in some embodiments, they can exhibit an ultimate tensile strength (UTS) between about 115 and 145 MPa as well as an electrical conductivity EC of at least 58% IACS.

The aluminum conductor alloys of the present disclosure can optionally comprise silicon (Si). In an embodiment, the aluminum conductor alloys comprise, in weight percent, up to about (e.g., a maximum of) 0.1 Si (in weight percent). In another embodiment, the aluminum conductor alloys comprise, in weight percent, up to about (e.g., a maximum of) 0.01, 0.02, 0.03, 0.04, 0.05, 0.06, 0.07, 0.08, 0.09 or 0.1 Si (in weight percent). In yet another embodiment, the aluminum conductor alloys comprise, in weight percent, up to about (e.g., a maximum of) 0.01, 0.02, 0.03, 0.04 or 0.05 Si (in weight percent). In still another embodiment, the aluminum conductor alloys comprise, in weight percent, up to about (e.g., a maximum of) 0.05 Si (in weight percent). In some embodiments, the aluminum conductor alloys comprise, in weight percent, about 0.05 Si (in weight percent).

The aluminum alloy of the present disclosure can optionally comprise iron (Fe). In an embodiment, the aluminum conductor alloys comprise, in weight percent, up to about (e.g., a maximum of) 0.5 Fe (in weight percent). In yet a further embodiment, the aluminum conductor alloys comprise, in weight percent, up to about (e.g., a maximum of) 0.1, 0.2, 0.3, 0.4 or 0.5 Fe (in weight percent). In yet a further embodiment, the aluminum conductor alloys comprise, in weight percent, up to about (e.g., a maximum of) 0.1, 0.2, 0.3 or 0.4 Fe (in weight percent). In yet a further embodiment, the aluminum conductor alloys comprise, in weight percent, up to about (e.g., a maximum of) 0.1, 0.2 or 0.3 Fe (in weight percent). In some embodiments, the aluminum alloys of the present disclosure comprise at least about (e.g., a minimum of) 0.3 Fe (in weight percent). In a further embodiment, the aluminum conductor alloys of the present disclosure comprise at least about 0.3 Fe and at up to about 0.4 or 0.5 Fe, for example, between about 0.3 Fe and about 0.4, between about 0.3 Fe and about 0.5 Fe (in weight percent). In embodiments in which improving the cast properties of the aluminum conductor alloy is preferred, the aluminum alloy comprises up to about 0.5 Fe or up to about 0.3 Fe (for example, between about 0.3 and about 0.5 Fe or between about 0.3 and about 0.4 Fe, in weight percent).

The aluminum conductor alloys of the present disclosure optionally comprise copper (Cu). The presence of Cu can increase primary creep resistance and can also increase ultimate tensile strength (UTS) in the resulting cast product. In an embodiment, the aluminum conductor alloys comprise up to about (e.g., a maximum of) 0.35 Cu (in weight percent). For example, the aluminum conductor alloys of the present disclosure can comprise up to about (e.g., a maximum of) 0.05, 0.06, 0.07, 0.08, 0.09, 0.10, 0.11, 0.12, 0.13, 0.14, 0.15, 0.16, 0.17, 0.18, 0.19, 0.20, 0.21, 0.22, 0.23, 0.24, 0.25, 0.26, 0.27, 0.28, 0.29, 0.30, 0.31, 0.32, 0.33, 0.34 or 0.35 Cu (in weight percent). In some embodiments, the

aluminum conductor alloys of the present disclosure comprise up to about (e.g., a maximum of) 0.30 Cu (in weight percent). For example, the aluminum conductor alloys can comprise up to about (e.g., a maximum of) 0.05, 0.06, 0.07, 0.08, 0.09, 0.10, 0.11, 0.12, 0.13, 0.14, 0.15, 0.16, 0.17, 0.18, 0.19, 0.20, 0.21, 0.22, 0.23, 0.24, 0.25, 0.26, 0.27, 0.28, 0.29 or 0.30 Cu (in weight percent). In an embodiment, the aluminum conductor alloys comprises between about 0.15 and about 0.30 Cu (in weight percent). In a further embodiment, the aluminum conductor alloys comprise at least about (e.g., a minimum of) 0.15, 0.16, 0.17, 0.18, 0.19, 0.20, 0.21, 0.22, 0.23, 0.24, 0.25, 0.26, 0.27, 0.28 or 0.29 Cu (in weight percent). In still another embodiment, the aluminum alloys comprise up to about (e.g., a maximum of) 0.30, 0.29, 0.28, 0.27, 0.26, 0.25, 0.24, 0.23, 0.22, 0.21, 0.20, 0.19, 0.18, 0.17 or 0.16 Cu (in weight percent). In yet another embodiment, the aluminum alloys comprise between about 0.15, 0.16, 0.17, 0.18, 0.19, 0.20, 0.21, 0.22, 0.23, 0.24, 0.25, 0.26, 0.27, 0.28 or 0.29 and about 0.30, 0.29, 0.28, 0.27, 0.26, 0.25, 0.24, 0.23, 0.22, 0.21, 0.20, 0.19, 0.18, 0.17 or 0.16 Cu (in weight percent). In an embodiment, the aluminum conductor alloys can comprise between about (e.g., a maximum of) 0.05, 0.06, 0.07, 0.08, 0.09, 0.1, 0.11, 0.12, 0.13, 0.14, 0.15, 0.16 or 0.17 and about 0.18, 0.17, 0.16, 0.15, 0.14, 0.13, 0.12, 0.11, 0.10, 0.09, 0.08, 0.07 or 0.06 Cu (in weight percent). In still another embodiment, the aluminum conductor alloys can comprise about 0.18 Cu (in weight percent).

The aluminum conductor alloys of the present disclosure comprise a deliberate addition of magnesium (Mg). As indicated above, the presence of Mg increases creep resistance in the resulting cast product. In an embodiment, the aluminum conductor alloys comprise up to about (e.g., a maximum of) 0.10 Mg, for example between about 0.02 and 0.10 Mg (in weight percent). For example, the aluminum conductor alloys of the present disclosure can comprise up to about (e.g., a maximum of) 0.02, 0.03, 0.04, 0.05, 0.06, 0.07, 0.08, 0.09 or 0.1 Mg (in weight percent). In some embodiments, the aluminum conductor alloys of the present disclosure comprise up to about (e.g., a maximum of) 0.1 Mg (in weight percent). In an embodiment, the aluminum conductor alloys comprises between about 0.02 to about 0.1 Mg (in weight percent). In a further embodiment, the aluminum conductor alloys comprise at least about (e.g., a minimum of) 0.02, 0.03, 0.04, 0.05, 0.06, 0.07, 0.08 or 0.09 Mg (in weight percent). In still another embodiment, the aluminum alloys comprise up to about (e.g., a maximum of) 0.1, 0.09, 0.08, 0.07, 0.06, 0.05, 0.04 or 0.03 Mg (in weight percent). In yet another embodiment, the aluminum alloys comprise between about 0.02, 0.03, 0.04, 0.05, 0.06, 0.07, 0.08 or 0.09 and about 0.1, 0.09, 0.08, 0.07, 0.06, 0.05, 0.04 or 0.03 Mg (in weight percent). In an embodiment, the aluminum conductor alloys can comprise up to about (e.g., a maximum of) 0.02, 0.03, 0.04, 0.05, 0.06, 0.07, 0.08 or 0.09 Mg (in weight percent). In still another embodiment, the aluminum conductor alloys can comprise about 0.052 Mg (in weight percent). In an embodiment, the aluminum conductor alloys can comprise up to about (e.g., a maximum of) 0.02, 0.021, 0.022, 0.023, 0.024 or 0.025 Mg (in weight percent). In still another embodiment, the aluminum conductor alloys can comprise about 0.025 Mg (in weight percent).

The aluminum conductor alloys of the present disclosure can optionally comprise boron (B). For example, the aluminum conductor alloys of the present disclosure can comprise between about 0.001 and about 0.04 B (in weight percent). In a further embodiment, the aluminum conductor alloys comprise at least about (e.g., a minimum of) 0.001,

0.002, 0.003, 0.004, 0.005, 0.006, 0.007, 0.008, 0.009, 0.01, 0.011, 0.012, 0.013, 0.014, 0.015, 0.016, 0.017, 0.018, 0.019, 0.02, 0.021, 0.022, 0.023, 0.024, 0.025, 0.026, 0.027, 0.028, 0.029, 0.03, 0.031, 0.032, 0.033, 0.034, 0.035, 0.036, 0.037, 0.038 or 0.039 B (in weight percent). In still another embodiment, the aluminum conductor alloys comprise up to about (e.g., a maximum of) 0.04, 0.039, 0.038, 0.037, 0.036, 0.035, 0.034, 0.033, 0.032, 0.031, 0.03, 0.029, 0.028, 0.027, 0.026, 0.025, 0.024, 0.023, 0.022, 0.021, 0.02, 0.019, 0.018, 0.017, 0.016, 0.015, 0.014, 0.013, 0.012, 0.011, 0.01, 0.009, 0.008, 0.007, 0.006, 0.005 or 0.004 B. In yet another embodiment, the aluminum conductor alloys comprise between about 0.003, 0.004, 0.005, 0.006, 0.007, 0.008, 0.009, 0.01, 0.011, 0.012, 0.013, 0.014, 0.015, 0.016, 0.017, 0.018, 0.019, 0.02, 0.021, 0.022, 0.023, 0.024, 0.025, 0.026, 0.027, 0.028 or 0.029 and about 0.03, 0.029, 0.028, 0.027, 0.026, 0.025, 0.024, 0.023, 0.022, 0.021, 0.02, 0.019, 0.018, 0.017, 0.016, 0.015, 0.014, 0.013, 0.012, 0.011, 0.01, 0.009, 0.008, 0.007, 0.006, 0.005, 0.004, 0.003 or 0.002 B (in weight percent).

The balance of the aluminum alloy of the present disclosure is aluminum (Al) and unavoidable impurities. In an embodiment, each impurity is present, in weight percent, at a maximum of about 0.03 and the total unavoidable impurities is present, in weight percent, at less than about 0.10 (in weight percent).

The aluminum conductor alloys of the present disclosure can be provided as rods. Rods can be cast from a continuous rod casting machine or from extruded billets. The rods can be worked into wires.

The aluminum conductor alloys of the present disclosure can be used in making electrical conductors. As indicated herein aluminum products, such as electrical conductors, comprising the aluminum conductor alloys of the present disclosure exhibit increased creep resistance in comparison with electrical conductors made from an aluminum conductor alloy comprising less than 0.02 Mg (in weight percent).

The present disclosure also provides a process for improving the creep resistance of an aluminum product when compared to a control aluminum product. In the context of the present disclosure, an improvement of the creep resistance refers to the reduction of the secondary creep rate. In an embodiment, the aluminum conductor alloys of the present disclosure exhibits a maximal secondary creep rate of at most  $1 \times 10^{-8}$  s at 100° C. under a 69 MPa load. In the process, the aluminum product is made from or comprises the aluminum alloy of the present disclosure (comprising at least about 0.02 Mg as a deliberate addition) whereas the control aluminum product is made from or comprises a first aluminum alloy (lacking Mg as a deliberate addition or having less than 0.02 Mg). The process comprises adding Mg (at the weight percent described above) to a first aluminum alloy (comprising Fe and Cu and optionally Si

and/or B, each at the weight percent described above) to provide the modified aluminum alloy (comprising Fe, Cu and Mg and optionally Si and/or B, each at the weight percent described above). In the context of the present disclosure, the term "aluminum product" can refer to a final cast products or to an intermediary rod which can further be worked into a differently shaped aluminum product. As such, the process can further comprise casting or working the aluminum conductor alloy into the aluminum product. In the embodiments in which the aluminum product is a cast product, the latter can be an electrical conductive material, such as an electrical conductor. The present disclosure also provides an aluminum product obtainable or obtained by the process described herewith.

The present disclosure also provides a process for making an aluminum product having an improved creep resistance when compared to a control aluminum product lacking a deliberate addition of Mg or having less than 0.02 Mg (in weight percent). The process comprises working the aluminum alloy or the modified aluminum conductor alloy described herewith or the rod described herewith into the aluminum product. The working step can include casting the aluminum alloy directly into a cast product or intermediary rods. As such, in the context of the present disclosure, the term "aluminum product" can refer to a final cast products or to an intermediary rod which can further be worked into a differently shaped aluminum product. In the embodiments in which the aluminum product is a cast product, the latter can be an electrical conductive material, such as an electrical conductor, a wire for example.

The present invention will be more readily understood by referring to the following examples which are given to illustrate the invention rather than to limit its scope.

#### Example I—Creep Resistance Determination

The materials used in this example were 8xxx aluminum alloys with three fixed Fe levels (Al-0.3Fe, Al-0.5Fe and Al-0.7Fe base alloys), alloyed with various Cu and Mg concentrations. The addition of 0.18% and 0.29% Cu were made to Al-0.3Fe, Al-0.5Fe and Al-0.7Fe base alloys, and further addition of 0.025%, 0.05% and 0.1% Mg were made to Al-0.3Fe-0.18Cu, Al-0.5Fe-0.18Cu and Al-0.7Fe-0.18Cu alloys, respectively. A total of 18 alloys with various Cu, Mg and Fe contents were batched in an electrical resistant furnace and cast in the form of round billets with 4 inches in diameter by a direct chill (DC) cast units. The chemical composition of each of the 18 alloys (L00 to H210) is shown in Table 1 (all alloy compositions are in wt. % unless otherwise indicated). All the rod samples with 9.5 mm in diameter, which are equivalent to the industrial 9.5 mm supply rods for drawn wire, were produced by the hot extrusion from DC cast billets.

TABLE 1

| Alloys                      | Chemical compositions of the experimental alloys investigated (wt. %) |      |       |       |       |       |       |      |
|-----------------------------|-----------------------------------------------------------------------|------|-------|-------|-------|-------|-------|------|
|                             | Fe                                                                    | Cu   | Mg    | Si    | Mn    | Cr    | Zn    | Al   |
| Al—0.3Fe (L00)              | 0.30                                                                  | 0.01 | 0.001 | 0.025 | 0.002 | 0.001 | 0.012 | Bal. |
| Al—0.3Fe—0.18Cu (L20)       | 0.30                                                                  | 0.18 | 0.001 | 0.023 | 0.003 | 0.001 | 0.002 | Bal. |
| Al—0.3Fe—0.29Cu (L30)       | 0.30                                                                  | 0.29 | 0.000 | 0.033 | 0.001 | 0.001 | 0.012 | Bal. |
| Al—0.3Fe0.18Cu—0.03Mg (L23) | 0.30                                                                  | 0.18 | 0.025 | 0.031 | 0.002 | 0.001 | 0.012 | Bal. |
| Al—0.3Fe0.18Cu—0.05Mg (L25) | 0.30                                                                  | 0.19 | 0.052 | 0.038 | 0.003 | 0.001 | 0.002 | Bal. |
| Al—0.3Fe0.18Cu—0.1Mg (L210) | 0.30                                                                  | 0.18 | 0.100 | 0.049 | 0.002 | 0.001 | 0.012 | Bal. |
| Al—0.5Fe (M00)              | 0.46                                                                  | 0.01 | 0.001 | 0.046 | 0.002 | 0.001 | 0.012 | Bal. |
| Al—0.5Fe—0.18Cu (M20)       | 0.50                                                                  | 0.18 | 0.001 | 0.027 | 0.004 | 0.001 | 0.002 | Bal. |

TABLE 1-continued

| Alloys                      | Fe   | Cu   | Mg    | Si    | Mn    | Cr    | Zn    | Al   |
|-----------------------------|------|------|-------|-------|-------|-------|-------|------|
| Al—0.5Fe—0.29Cu (M30)       | 0.47 | 0.29 | 0.000 | 0.023 | 0.002 | 0.001 | 0.003 | Bal. |
| Al—0.5Fe0.18Cu—0.03Mg (M23) | 0.46 | 0.18 | 0.026 | 0.051 | 0.002 | 0.001 | 0.013 | Bal. |
| Al—0.5Fe0.18Cu—0.05Mg (M25) | 0.44 | 0.17 | 0.055 | 0.021 | 0.001 | 0.001 | 0.002 | Bal. |
| Al—0.5Fe0.18Cu—0.1Mg (M210) | 0.47 | 0.18 | 0.100 | 0.049 | 0.002 | 0.001 | 0.012 | Bal. |
| Al—0.7Fe (H00)              | 0.70 | 0.01 | 0.001 | 0.023 | 0.002 | 0.001 | 0.013 | Bal. |
| Al—0.7Fe—0.18Cu (H20)       | 0.70 | 0.19 | 0.001 | 0.042 | 0.003 | 0.001 | 0.016 | Bal. |
| Al—0.7Fe—0.29Cu (H30)       | 0.71 | 0.29 | 0.000 | 0.032 | 0.003 | 0.001 | 0.002 | Bal. |
| Al—0.7Fe0.18Cu—0.03Mg (H23) | 0.69 | 0.18 | 0.027 | 0.052 | 0.002 | 0.001 | 0.013 | Bal. |
| Al—0.7Fe0.18Cu—0.05Mg (H25) | 0.70 | 0.18 | 0.056 | 0.042 | 0.003 | 0.001 | 0.012 | Bal. |
| Al—0.7Fe0.18Cu—0.1Mg (H210) | 0.72 | 0.18 | 0.100 | 0.051 | 0.002 | 0.001 | 0.013 | Bal. |

15

The electrical conductivity measurement was directly conducted on the samples of 9.5 mm in diameter and 200 mm long using Megger DLRO10HD resistance ohmmeter. Tensile test was carried out on cylindrical specimens (9.5 mm in diameter and 250 mm in length) according to ASTM B557 standard at room temperature. The compression creep tests were conducted on cylindrical specimens (with a diameter of 9.5 mm and a length of 19 mm) at 100°C for 100 hours under a constant load 69 MPa. To confirm the reliability of the results, 3 tests were repeated for each condition.

For microstructure examination, the extruded rods were first cut 20 mm in length and then sectioned longitudinally along the centerline. All the samples were polished and etched by the Keller's solution for 10 seconds and then were observed using optical microscope (OM), scanning electron microscope (SEM) and electron backscattered diffraction (EBSD) technique. The automated EBSD maps were conducted on the deformed structure with step size of 0.2  $\mu\text{m}$  using HKL Channel 5 software for substructure analysis. The linear intercept method (as described in F. J. Humphreys, J. Mater. Sci. 36 (2001) 3833-3854, C. J. Shi, W. M. Mao, X. G. Chen, Mater. Sci. Eng. A 571 (2013) 83-91) was used to measure the subgrain size of alloys with different alloying contents. To ensure statistical reliability, more than 200 subgrains were measured in each sample.

Microstructure evolution. FIGS. 1(A) to 1(D) show optical micrographs of some typical alloys with different compositions after extrusion ((A) Al-0.3Fe, (B) Al-0.3Fe-0.29Cu, (C) Al-0.7Fe, and (D) Al-0.7Fe0.18Cu-0.1Mg). Due to a very low solubility of Fe in aluminum matrix, almost all the Fe precipitated out in the form of Fe-contained intermetallic networks in the cast microstructure. During hot extrusion, the Fe-contained intermetallic networks were broken down to a number of fine intermetallic dispersion particles. For all the alloys, the fine intermetallic particles, which were confirmed as  $\text{Al}_m\text{Fe}$ , were uniformly distributed along the extrusion direction in aluminum matrix. With increasing amount of Fe, from 0.3 to 0.7%, in the three base alloys (Al-0.3Fe, Al-0.5Fe, Al-0.7Fe), the volume fraction of Fe-contained intermetallic particles was increased from 1.8% in Al-0.3Fe to 3.2% in Al-0.5Fe and further to 4.4% in Al-0.7Fe alloys. When Cu and Mg were added to the three base alloys, the volume fraction of intermetallic particles were found to remain approximately unchanged compared to the corresponded base alloys. A comparison of FIGS. 1(A) and (B) shows the evolution of the particles distribution of the alloys for the addition of 0.29% Cu, and a comparison of FIGS. 1(C) and (D) shows the evolution of the particles distribution of the alloys for the combined addition of 0.18% Cu and 0.1% Mg. Without wishing to be

bound to theory, this can be attributed to the higher solid solubility of Cu and Mg in aluminum, which is approximately 0.4% and 1.7% at room temperature, respectively. Therefore, Cu up to 0.29% and Mg up to 0.1% were expected to remain all in the solid solution after extrusion. On the other hand, the size of Fe-contained intermetallic particles was measured to be similar with an average value of 0.38  $\mu\text{m}$  for all the alloys studied.

To understand the microstructure evolution with additions of Cu and Mg in 8xxx aluminum alloys, EBSD orientation maps of the same typical alloy samples as in FIG. 1 were examined. All the extruded alloys showed a characteristic of recovered structure (data not shown). A large amount of low-angle boundaries with misorientation angles between of 1° and 5° were observed, indicating a number of cells and subgrains. In addition, the substructures were organized and large well-defined subgrains were formed along the elongated grains with neatly arranged boundaries of 1-15°, suggesting that dynamic recovery happened, thereby involving the annihilation and rearrangement of dislocations.

Though the recovered structure was present in all experimental alloys, differences in subgrain size were observed due to additions of Cu and Mg. In the present example, the average subgrain size was measured from the EBSD orientation maps and the results are illustrated in FIG. 2. It was found that the average subgrain size was decreased from 4.5  $\mu\text{m}$  in Al-0.3Fe to 3.7  $\mu\text{m}$  in Al-0.5Fe and further to 3.2  $\mu\text{m}$  in Al-0.7Fe as the amount of Fe increased from 0.3% to 0.7% in the base alloys. On the other hand, with increasing Cu (0.18-0.29%), the subgrain size slightly decreased from 4.5 to 3.8  $\mu\text{m}$  in Al-0.3Fe—Cu, from 3.7 to 3.3  $\mu\text{m}$  in Al-0.5Fe—Cu and from 3.2 to 2.7  $\mu\text{m}$  in Al-0.7Fe—Cu alloys (FIG. 2(A)), respectively. However, a further addition of Mg (0.025-0.1%) in all three base alloys showed almost no effect on subgrain size (FIG. 2(B)). Without wishing to be bound to theory, the decrease of the subgrain size with increasing Fe content in the base alloys can be interpreted by the increase of the volume fraction of Fe-contained intermetallic particles, which had strong pinning effect on dislocation motion and subgrain growth. Besides, Cu solutes in aluminum solution have a lower diffusion rate than for aluminum self-diffusion, which would strongly hinder the dislocation movement at the subgrain boundaries and enhance dislocation multiplication, leading to the retardation of the dynamic recovery. However, the diffusion rate of Mg is very close to aluminum self-diffusion, which resulted in little effect on the dynamic recovery. As a result, with increasing Cu level the subgrain size decreased while the Mg addition exhibited no effect on subgrain size.

Effects of Cu and Mg on electrical conductivity and ultimate tensile strength. FIG. 3 shows the evolution of the

electrical conductivity (EC) with different amounts of Cu and Mg in 8xxx aluminum alloys. It was found that EC slightly decreased with increasing Cu and Mg due to enhanced scattering of free electrons at Cu and Mg solutes in aluminum. With increasing Cu from 0 to 0.29%, EC decreased from 62.4 to 60.5% IACS in Al-0.3Fe—Cu alloy and from 60.9 to 59.1% IACS in Al-0.7Fe—Cu alloy (FIG. 3(A)), while with increasing Mg from 0% to 0.1%, EC decreases from 61.1 to 60.2% IACS in Al-0.3Fe0.18Cu—Mg alloy and from 59.7 to 58.8% IACS in Al-0.7Fe0.18Cu—Mg alloy (FIG. 3(B)), respectively.

In order to quantitatively analyze the experimental data, a Matthiessen's law (as described in B. Raeisnia, W. J. Poole, D. J. Lloyd, Mater. Sci. Eng. A 420 (2006) 245-249) was adapted to establish the relationship of the EC with chemical composition as follows:

$$\frac{1}{EC} = \rho_b + \sum_i \rho_i C_i + \rho_p f_p \quad (Eq. 1)$$

where EC is the electrical conductivity,  $\rho_b$  is resistivity of the base alloy,  $\sum_i \rho_i C_i$  is the sum of the resistivity contributions from the various solution additions, i.e.  $\rho_i$  is the resistivity parameter and  $C_i$  is the concentration of the  $i^{th}$  solute,  $\rho_p$  is the resistivity parameter of the particles to resistivity and  $f_p$  is the particle volume fraction. In the present example, due to the low solubility of Fe in aluminum, it can be assumed that almost all the Fe precipitated out into intermetallic particles and the volume fraction of intermetallic particles has a close and linear relation with Fe contents. As all the alloys had similar particles size, the particle contribution  $\rho_p f_p$  in Eq. 1 can be substituted by  $\rho'_{Fe} C_{Fe}$ . Consequently, Eq. 1 can be transformed to:

$$\frac{1}{EC} = \rho_b + \rho_{Cu} C_{Cu} + \rho_{Mg} C_{Mg} + \rho'_{Fe} C_{Fe} \quad (Eq. 2)$$

where EC is in the unit of % IACS,  $\rho_{Cu}$ ,  $\rho_{Mg}$  and  $\rho'_{Fe}$  are the resistivity parameters of Cu, Mg and Fe alloying elements, and  $C_{Cu}$ ,  $C_{Mg}$  and  $C_{Fe}$  are the concentrations in wt. %. Based on the results from FIG. 3, the values of all resistivity parameters ( $\rho$ ) can be obtained using the multiple linear regression method. Subsequently, an empirical expression can be obtained to predict the electrical conductivity as a function of alloying element contents:

$$1/EC = 0.01575 + 0.00174 C_{Cu} + 0.00289 C_{Mg} + 0.00096 C_{Fe} \quad (Eq. 3)$$

Using Eq. 3, the values of EC can be calculated with different Cu, Mg and Fe contents for 8xxx aluminum alloys. In the present example, the calculated values of the electrical conductivity versus the measured values with different Cu and Mg contents in the three base alloys are plotted in FIG. 4 (Al-0.3Fe—Cu—Mg, Al-0.5Fe—Cu—Mg, Al-0.7Fe—Cu—Mg). As demonstrated, there is excellent agreement between the calculated and experimental results. Furthermore, to evaluate the accuracy of the equation 3, the error between the calculated EC(C) and the measured EC(M) can be expressed as follows:

$$Error \% = \left| \frac{EC(C) - EC(M)}{EC(M)} \right| 100 \quad (Eq. 4)$$

The mean error for the 8xxx alloys with Cu contents (ranging from 0% to 0.29%) and Mg contents (ranging from 0% to 0.1%) was determined to be 0.13%, which confirms again an excellent agreement between the predicted and measured EC. Therefore, the obtained equation 3 offers a very good prediction of the electrical conductivity as function of alloying elements (Cu, Mg and Fe) in 8xxx aluminum alloys.

On the other hand, the UTS of the alloys were evaluated with different compositions and the results are shown in Table 2. It was found that UTS was moderately increased with increasing Cu and Mg concentrations most likely due to solid solution strengthening and substructure strengthening. The results also reveal a beneficial effect of Cu and Mg on the mechanical properties. Besides, the UTS showed a nearly linear relationship with Cu, Mg and Fe contents, as shown in FIG. 5. The overall strength  $\sigma$  (UTS) of the alloys can be expressed by an empirical equation in the form (as described in E. A. Marquis, D. N. Seidman, D. C. Dunand, Acta Mater. 51 (2003) 4751-4760 and R. A. Karnesky, L. Meng, D. C. Dunand, Acta Mater. 55 (2007) 1299-1308):

$$\sigma(UTS) = \sigma_b + H_{Cu} C_{Cu} + H_{Mg} C_{Mg} + H_{Fe} C_{Fe} \quad (Eq. 5)$$

where  $\sigma_b$  is strength of the base alloy in the unit of MPa,  $H_{Cu}$ ,  $H_{Mg}$  and  $H_{Fe}$  are the strengthening parameters of Cu, Mg and Fe, and  $C_{Cu}$ ,  $C_{Mg}$  and  $C_{Fe}$  are the concentrations in wt. %. By using the multiple linear regression method, the value of ab and strengthening parameters (H) were determined to be 75.6 for  $\sigma_b$ , 51.1 for  $H_{Cu}$ , 66.7 for  $H_{Mg}$  and 71.0 for  $H_{Fe}$ , respectively. Then, the equation can be used to describe the UTS as a function of alloying element contents:

$$UTS = 75.6 + 51.1 C_{Cu} + 66.7 C_{Mg} + 71.0 C_{Fe} \quad (Eq. 6)$$

According to Eq. 6, the values of UTS with different Cu, Mg and Fe contents can be calculated. The calculated values of the UTS versus the measured values for the 8xxx alloys with various Cu, Mg and Fe contents in different base alloys were plotted in FIG. 6, which demonstrated good agreement between the calculated and experimentally measured results. Besides, the mean error between the calculated UTS(C) and the measured UTS(M) for the 8xxx alloys with addition of Cu (0-0.29%) and Mg (0-0.1%) was determined to be 1.0%, which confirmed the agreement between the calculated and measured UTS. Therefore, the obtained equation 6 could be used to calculate the UTS of 8xxx aluminum alloys after alloying with various Cu, Mg and Fe additions.

TABLE 2

| The variations of UTS with Cu and Mg in different base alloys. |           |        |           |        |           |
|----------------------------------------------------------------|-----------|--------|-----------|--------|-----------|
| Alloys                                                         | UTS (MPa) | Alloys | UTS (MPa) | Alloys | UTS (MPa) |
| 50                                                             | 98.2      | M00    | 107.5     | H00    | 126.8     |
|                                                                | 107.7     | M20    | 116.7     | H20    | 134.2     |
|                                                                | 113.2     | M30    | 122.2     | H30    | 141.6     |
|                                                                | 108.5     | M23    | 117.3     | H23    | 138.2     |
|                                                                | 109.7     | M25    | 119.7     | H25    | 138.3     |
|                                                                | 113.5     | M210   | 123.3     | H210   | 142.8     |

From Eqs. 3 and 6, the EC and UTS could be quantitatively calculated according to Cu, Mg and Fe contents. For aluminum conductor alloys, high EC with enhanced UTS are most desirable properties in 8xxx aluminum alloys. However, high EC and high UTS are usually opposite because of the metallurgical nature of both properties. The EC and UTS profile of the alloys with different Cu and Mg additions in Al-0.3Fe, Al-0.5Fe and Al-0.7Fe base alloys were plotted in FIG. 7. This figure can be divided into three

regions with different combinations of EC and UTS. The region I is with high UTS but low EC while the region III is with high EC but low UTS. The region II in the middle has a balanced EC and UTS. In the present study, both 0.3Fe (L00) and 0.5Fe (M00) alloys have higher EC but lower UTS (region III) compared to 0.7Fe (H00) alloy (region II). With additions of Cu and Mg, 0.3Fe and 0.5Fe alloys moved to the region II with a balanced EC and UTS. For example, 0.5Fe alloys with Cu and Mg additions could possibly have a similar value of EC and UTS compared with 0.7Fe (H00) alloy. It is also evident that 0.7 alloys with Cu and Mg additions tend to move from the region I to the region II, which have higher UTS but relatively lower EC. By adjusting Fe and Cu and Mg alloying elements, different combinations of EC and UTS could be obtained to fulfill different design requirements for specific product applications.

Effects of Cu and Mg on creep properties. FIG. 8 shows typical creep strain ( $\epsilon$ ) and instantaneous creep rate ( $d\epsilon/dt$  or  $\dot{\epsilon}$ ) curves of Al-0.3Fe alloys with Cu additions, tested at 100° C. under a constant load of 69 MPa. It can be seen that the total creep strain greatly decreases from 6.87% in Al-0.3Fe base alloy to 2.44% in Al-0.3Fe-0.29Cu alloy (FIG. 8(A)). In general, during the compressive creep deformation, the creep strain rapidly increases with increasing time at the beginning of creep deformation due to an initial high rate of work hardening (defined as the primary stage, where  $d\epsilon/dt < 0$ ). Subsequently, the creep deformation runs to a quasi-steady state, in which the creep rate,  $d\epsilon/dt$ , becomes more and less constant (namely the second stage,  $d\epsilon/dt \approx 0$ ). It is suggested the second stage dominates the creep deformation during the long-term creep process. As shown in FIG. 8(B), the minimum creep rate ( $\dot{\epsilon}_m$  in  $s^{-1}$ ) is calculated as the average creep rate in the second stage, and the results show that with increasing Cu content from 0% to 0.29%, the  $\dot{\epsilon}_m$  slightly decreased from  $8.1 \times 10^{-8}$  to  $6.1 \times 10^{-8} s^{-1}$ . The results from FIG. 8 indicated that addition of Cu was mainly beneficial at the primary creep stage but has very little effect at second creep stage.

FIG. 9 shows typical creep strain ( $\epsilon$ ) and instantaneous creep rate ( $d\epsilon/dt$  or  $\dot{\epsilon}$ ) curves of Al-0.3Fe-0.18Cu alloys with different amounts of Mg. Similarly as FIG. 8, the compressive creep curve consists of the primary creep stage and the second stage. As shown on FIG. 9(A), it can be found that the total creep strain considerably decreases with increasing Mg content and the value decreases from 4.17% in the base alloy (Al-0.3Fe-0.18Cu) to 0.14% in the 0.1% Mg containing alloy (Al-0.3Fe-0.18Cu-0.1Mg). On the other hand, as shown in FIG. 9(B), with increasing Mg from 0% to 0.1%, the  $\dot{\epsilon}_m$  significantly decreases from  $7.5 \times 10^{-8} s^{-1}$  in the base alloy to  $4.8 \times 10^{-10} s^{-1}$  with the 0.1% Mg containing alloy, indicating a strong and positive effect of Mg on improving the minimum creep rate. It is suggested that addition of Mg was beneficial to largely enhance the creep property both at the primary creep stage and second stage.

From the creep strain ( $\epsilon$ ) and creep rate ( $d\epsilon/dt$  or  $\dot{\epsilon}$ ) curves as shown in FIGS. 8 and 9, it is noted that additions of Cu and Mg showed different impact on the creep resistance of 8xxx aluminum alloys. To better understand the Cu and Mg effect, the evolution of the primary creep strain ( $\epsilon_p$ ) and minimum creep rate as a function of Cu and Mg contents was evaluated, as shown in FIG. 10. The primary creep strain  $\epsilon_p$  is obtained by extrapolating the second creep curve linearly back to the zero time (X. W. Wei, X. T. Zu, W. L. Zhou, Mater. Sci. Tech. 22 (2006) 730-733), as illustrated by the dotted line in FIG. 8(A). As indicated in FIGS. 10(A) and (B), the primary creep strain  $\epsilon_p$  was significantly decreased with increasing Cu and Mg content. With increasing Cu

from 0% to 0.29% in weight percent (FIG. 10(A)), the primary creep strain decreased from 3.82% to 0.43% in Al-0.3Fe-Cu alloys (89% reduction), from 1.25% to 0.22% in Al-0.5Fe-Cu alloys (82% reduction), and from 0.71% to 0.15% in Al-0.7Fe-Cu alloys (79% reduction), respectively. As shown in FIG. 10(B), when Mg increases from 0% to 0.1% (in weight percent), the primary creep strain ( $\epsilon_p$ ) greatly decreased from 1.37% to 0.09% in Al-0.3Fe-0.18Cu-Mg alloys (93% reduction), from 0.43% to 0.07% in Al-0.5Fe-0.18Cu-Mg alloys (84% reduction), and from 0.25% to 0.05% in Al-0.7Fe-0.18Cu-Mg alloys (80% reduction). The results indicated the positive effect of both minor Cu and Mg additions on primary creep strain.

The evolution of minimum creep rate ( $\dot{\epsilon}_m$ ) as a function of Cu and Mg content is illustrated in FIGS. 10(C) and (D). It is interesting to notice that addition of Cu had almost no effect on the minimum creep rate while Mg remarkably decreased the minimum creep rate. With increasing Mg content from 0% to 0.1% (FIG. 10(D)), the minimum creep rate noticeably decreases from  $7.5 \times 10^{-8} s^{-1}$  to  $4.8 \times 10^{-10} s^{-1}$  in Al-0.3Fe-0.18Cu-Mg alloys (99% reduction), and from  $1.8 \times 10^{-8} s^{-1}$  to  $2.8 \times 10^{-10} s^{-1}$  in Al-0.3Fe-0.18Cu-Mg alloys (98% reduction) and further from  $5.6 \times 10^{-9} s^{-1}$  to  $2.1 \times 10^{-10} s^{-1}$  in Al-0.3Fe-0.18Cu-Mg alloys (96% reduction), respectively.

Although additions of minor Cu and Mg can considerably improve the creep properties, individual alloying elements can have different impacts. Firstly, with increasing Cu, the subgrain size slightly decreased, which can moderately retard the dislocation movement and thus decreases the primary creep strain. Moreover, the solid solution strengthening of Cu should be principally responsible for the significant decrease of the primary creep strain, because the Cu solutes increase the work hardening ability of the material. On the other hand, the results show that the minor addition of Cu had no effect on the minimum creep rate during the second creep stage, which is probably due to low interaction between the dislocation and Cu solute atmosphere. Without wishing to be bound to theory, those results suggested that the Cu addition could be effective in increasing creep resistance during the short-term creep deformation, where the primary creep stage plays an important role. Conversely, the Cu addition may not offer an advantage to the creep resistance under the long-term creep deformation.

The minor addition of Mg (0.025-0.1%) in 8xxx aluminum alloy seems not to have obvious effect on the deformed microstructure as shown in FIG. 2. However, it can considerably decrease both the primary creep strain ( $\epsilon_p$ ) and minimum creep rate ( $\dot{\epsilon}_m$ ), resulting in a significant improvement on the creep properties.

It is worthwhile mentioning that the effect of Cu and Mg on the creep property was decreased with increasing Fe in the base alloys, as shown in FIG. 10. Cu and Mg addition are believed to be more effective in increasing the creep property of 8xxx aluminum alloys in low Fe conditions.

In conclusion, the addition of Cu promoted the retardation of the dynamic recovery, which leads to a finer subgrain size. However, the addition of Mg showed little effect on the retardation of the dynamic recovery. The additions of Cu and Mg reasonably increased the UTS but slightly decreased EC. The effects of Cu, Mg and Fe on the UTS and EC were quantitatively evaluated and summarized in Eqs. 3 and 6, which offer a good prediction of the UTS and EC as a function of alloying elements (Cu, Mg and Fe) in 8xxx aluminum conductor alloys. The addition of Cu remarkably decreases the primary creep strain ( $\epsilon_p$ ) and shows almost no effect on the minimum creep rate ( $\dot{\epsilon}_m$ ), leading to a beneficial

## 15

effect on the early creep deformation but no advantage to the creep resistance under the long-term creep process. The minor addition of Mg greatly reduced both primary creep strain and minimum creep rate, resulting in a significant and effective improvement on the creep resistance of 8xxx aluminum conductor alloys.

## Example II—Casting Properties

The materials used in this example were various aluminum alloys as shown in Table 3 (all alloy compositions are in wt. % unless otherwise indicated). The alloys were batched in a 100 tons furnace and cast on a continuous rod casting machine. Liquid metal is solidified in a rectangular bar which is immediately rolled into a 9.5 mm rod.

TABLE 3

| Chemical compositions of the experimental alloys investigated (wt. %) |      |      |    |      |         |
|-----------------------------------------------------------------------|------|------|----|------|---------|
| Alloys                                                                | Fe   | Cu   | Mg | Si   | Al      |
| 1                                                                     | 0.69 | 0.18 | —  | 0.05 | Balance |
| 2                                                                     | 0.55 | 0.01 | —  | 0.05 | Balance |
| 3                                                                     | 0.35 | 0.17 | —  | 0.05 | Balance |
| 4                                                                     | 0.16 | —    | —  | 0.05 | Balance |

The bar temperature, used as surrogate marker for the casting efficiency, was determined using thermocouple and/or pyrometer. As shown in FIG. 11, aluminum conductor alloys having 0.5 or less Fe exhibit a decreased bar temperature and are thus considered to be casted more efficiently.

While the invention has been described in connection with specific embodiments thereof, it will be understood that the scope of the claims should not be limited by the preferred embodiments set forth in the examples, but should be given the broadest interpretation consistent with the description as a whole.

What is claimed is:

1. An aluminum conductor alloy having increased creep resistance, the aluminum conductor alloy comprising, in weight percent:  
up to about 0.10 Si;  
up to about 0.5 Fe;  
up to about 0.30 Cu;  
between about 0.021 and about 0.025 Mg;  
up to about 0.04 B; and  
the balance being aluminum and unavoidable impurities.
2. The aluminum conductor alloy of claim 1, comprising up to about 0.05 Si, in weight percent.
3. The aluminum conductor alloy of claim 1, comprising between about 0.3 and about 0.5 Fe, in weight percent.
4. The aluminum conductor alloy of claim 1, comprising between about 0.15 and about 0.30 Cu, in weight percent.
5. The aluminum alloy of claim 4, comprising up to about 0.18 Cu, in weight percent.

## 16

6. The aluminum alloy of claim 1, comprising between about 0.001 and about 0.04 B, in weight percent.

7. The aluminum alloy of claim 1, having a secondary creep rate of  $1 \times 10^{-8} \text{ s}^{-1}$  or less when measured at 100° C. under a 69 MPa load.

8. A rod comprising the aluminum conductor alloy of claim 1.

9. An aluminum cast product comprising the aluminum conductor alloy of claim 1.

10. The process of claim 1, wherein the modified aluminum conductor alloy comprises between about 0.15 and about 0.30 Cu, in weight percent.

11. The process of claim 10, wherein the modified aluminum conductor alloy comprises up to about 0.18 Cu, in weight percent.

12. A process for improving the creep resistance of an aluminum product comprising a modified aluminum conductor alloy when compared to a corresponding aluminum product comprising a first aluminum conductor alloy, the process comprising combining Mg with the first aluminum conductor alloy to provide the modified aluminum conductor alloy, wherein the first aluminum conductor alloy comprises, in weight percent:

up to about 0.10 Si;  
up to about 0.5 Fe;  
up to about 0.30 Cu;  
up to about 0.04 B; and  
the balance being aluminum and unavoidable impurities; wherein the modified aluminum alloy comprises between about 0.021 and about 0.025 Mg.

13. The process of claim 12, wherein the modified aluminum conductor alloy comprises up to about 0.05 Si, in weight percent.

14. The process of claim 12, wherein the modified aluminum conductor alloy comprises between about 0.3 and about 0.5 Fe, in weight percent.

15. The process of claim 12, wherein the modified aluminum conductor alloy comprises between about 0.001 and about 0.04 B, in weight percent.

16. The process of claim 12, wherein the modified aluminum conductor alloy has a secondary creep rate of  $1 \times 10^{-8} \text{ s}^{-1}$  or less when measured at 100° C. under a 69 MPa load.

17. An aluminum conductor alloy having increased creep resistance, the aluminum conductor alloy consisting essentially of, in weight percent:

up to about 0.10 Si;  
up to about 0.5 Fe;  
up to about 0.30 Cu;  
between about 0.021 and about 0.025 Mg;  
up to about 0.04 B; and  
the balance being aluminum and unavoidable impurities.

18. The aluminum conductor alloy of claim 17, wherein the aluminum conductor alloy contains between about 0.001 and about 0.04 B, in weight percent.

\* \* \* \* \*